# EUROPEAN PATENT APPLICATION

(11) **EP 4 230 755 A1**
(43) Date of publication of application: **23.08.2023**
(21) Application number: 22158008.7
(22) Date of filing: 22.02.2022
(51) Int. Cl.: C22C 1/02, C22C 21/06, C22F 1/047, C22C 21/08

(54) **ALLOY CONTAINING ALUMINIUM FOR EXTRUSION OR OTHER WROUGHT MANUFACTURING PROCESS**

(71) Applicant: Fehrmann GmbH, 21107 Hamburg (DE)
(72) Inventor: FRANKE, Rüdiger, 21107 Hamburg (DE); MONTEIRO, Antonio, 21107 Hamburg (DE); FEHRMANN, Henning, 21107 Hamburg (DE)
(74) Representative: Maiwald GmbH

(57) **Abstract**

The present invention relates to an alloy containing aluminium and magnesium, a method for the manufacture of said alloy, a method for the manufacture of a product comprising said alloy, a product comprising said alloy, and in particular to the use of said alloy in an extrusion or other wrought manufacturing process.

## Description

### Field of the Invention

The present disclosure relates to an alloy containing aluminium and magnesium, a method for the manufacture of said alloy, a method for the manufacture of a product comprising said alloy, a product comprising said alloy, and in particular to the use of said alloy in an extrusion or other wrought manufacturing process.

### Background

Extrusion processes are used as forming process for a variety of aluminium products, such as rods, wires, tubes, hollow profiles, solid profiles, and irregularly shaped prismatic profiles.

Such products desirably have high elongation combined with high strength. Such properties provide for excellent energy uptake capacity of the aluminium products. Therefore, such aluminium products find application in automotive industry, e.g., in the manufacture of mechanically stable parts of a car to provide increased crash safety for the passengers. Further applications of extruded aluminium products may be in aircraft engineering, shipbuilding, train construction, and the construction sector.

A crucial aspect in the manufacturing of aluminium products by means of extrusion processes is the aluminium alloy. Such alloy must have a coarse grain structure to provide for sufficient deformation characteristics, i.e. good formability, which are essential for successful extrusion. It is understood that the microstructure of an aluminium alloy is refined during forming by an extrusion process. This results in a refined microstructure of the aluminium product and hence increased strength and elongation properties.

Therefore, it is understood that aluminium alloys used in casting applications or the like are not suitable for application in extrusion processes: Such alloys are generally designed to provide high strength after casting. However, this means that high forces are required during extrusion which exceed the limits imposed by the available extrusion presses and plants.

Another important parameter in forming of aluminium alloys by extrusion is the extrusion temperature, the level of which is limited by the respective alloy composition, in particular by its resistance to heat impact. Since local heating of the alloy can occur during forming, melting can occur, especially in the region of the die, which impairs the mechanical properties of the final extruded product.

In conclusion, the design possibilities in extrusion are mainly influenced and limited by the type of alloy, the available process forces and the direction of extrusion. The advantages of extrusion are in particular the possibilities of producing profiles even in complex shapes. The high degree of forming that can be achieved in one process step and the low tooling costs make extrusion particularly interesting for the production of relatively small batches.

In the prior art, a variety of metals and alloys are described to be suitable for the manufacture of products by means of extrusion or wrought processes, including aluminium and aluminium alloys which are manufactured into heat sink profiles and construction profiles. Frequently, copper and copper alloys or stainless steel is used to produce seamless tubes.

The quality of the extruded part depends not only on the machine settings and the tool design (geometry) but also to a large extent on the alloy system selected. Predominantly, AlMn(Cu) alloys from the 2000 or 5000 series alloys according to the International Alloy Designation System and AIMgSi alloy systems from the 6000 series alloys according to the International Alloy Designation System are widely used for extruded products. The chemical composition and microstructure of an aluminium alloy is a decisive parameter in the manufacturing of aluminium products by means of extrusion processes for the resulting product properties.

Usually, the required mechanical properties, especially a high strength in terms of yield strength Rₘ and tensile strength R_{p0.2} are achieved by adding copper and/or zinc to the alloys. In addition, these alloys are subjected to a heat treatment in order to achieve an improvement of the mechanical properties through the hardening effects. In this process, metastable phases are formed to counteract dislocation movements when force is applied. Alternatively, Al-Mn alloys (3000 series alloys according to the International Alloy Designation System) may also be used.

### Summary of the Disclosure

There is still a need for an aluminium alloy that may be used in extrusion and/or wrought processes, allowing for the convenient manufacture of aluminium products having good mechanical properties, in particular all of good tensile strength, good yield strength and good elongation combined.

It has now been surprisingly found out that the aluminium alloys of the present disclosure have good mechanical properties, in particular high tensile strength, high yield strength and high elongation, while allowing the use of the alloy in manufacturing of products by means of extrusion and/or wrought processes.

In a first aspect, the present disclosure relates to an aluminium alloy comprising
a) of from 6 to 12 % by mass of magnesium (Mg);
b) of from 0.01 to 0.5 % by mass of titanium (Ti);
c) of from 0.001 to 0.1 % by mass of boron (B);
d) of from 0.002 to 0.2 % by mass of beryllium (Be);
e) of from 0 to 2.5 % by mass of manganese (Mn);
f) of from 0 to 0.2 % by mass of iron (Fe);
g) of from 0 to 5 % by mass of zinc (Zn);
h) of from 0 to 1 % by mass of chromium (Cr);
i) of from 0 to 1 % by mass of zirconium (Zr);
j) of from 0 to 0.5 % by mass of vanadium (V);
k) of from 0 to 0.06 % by mass of copper (Cu);
l) of from 0 to 1 % by mass of silicon (Si);
m) of from 0 to 1 % by mass of nickel (Ni);
n) of from 0 to 0.5 % by mass of cobalt (Co);

wherein the aluminium alloy further comprises inevitable impurities;
with the balance being aluminium (Al);
each amount in relation to the total mass of the alloy composition, and wherein all compounds of the aluminium alloy add up to a total of 100 % by mass.

In a second aspect, the present disclosure relates to an aluminium alloy product comprising an aluminium alloy according to the first aspect as disclosed above.

A third aspect of the present disclosure relates to a method for the manufacture of an aluminium alloy according to the first aspect as disclosed above, comprising the steps of
a) Providing a raw aluminium;
b) Heating the raw aluminium to a temperature in the range of from 650 to 850 °C, preferably from 750 to 800 °C;
c) Adding Mg and Be to result in a raw alloy;
d) Optionally degassing the raw alloy;
e) Adding Ti and B to the optionally degassed raw alloy to prepare the aluminium alloy; and
f) Casting the aluminium alloy to prepare an aluminium billet.
   In a fourth aspect, the present disclosure relates to a method for the manufacture of an aluminium alloy product according to the second aspect as disclosed above, wherein the manufacture of the aluminium alloy product comprises the steps of
g) Preheating an aluminium billet of an aluminium alloy according to the first aspect as disclosed above, to a temperature in the range of from 400 °C to 450 °C to result in a preheated aluminium billet;
h) Inserting the preheated aluminium billet from step g) into an extrusion press;
i) Extruding the preheated aluminium billet to result an extruded aluminium profile.

In a fifth aspect, the present disclosure relates to an extruded aluminium profile prepared by a method according to the fourth aspect as disclosed above.

In a sixth aspect, the present disclosure relates to the use of an aluminium alloy according to the first aspect disclosed herein in an extrusion process or a wrought process.

### Short Description of Figures

- Figure 1:: Schematic drawing of an aluminium hollow profile

### Detailed Description

### The Aluminium Alloy

In a first aspect, the present disclosure relates to an aluminium alloy comprising
a) of from 6 to 12 % by mass of magnesium (Mg);
b) of from 0.01 to 0.5 % by mass of titanium (Ti);
c) of from 0.001 to 0.1 % by mass of boron (B);
d) of from 0.002 to 0.2 % by mass of beryllium (Be);
e) of from 0 to 2.5 % by mass of manganese (Mn);
f) of from 0 to 0.2 % by mass of iron (Fe);
g) of from 0 to 5 % by mass of zinc (Zn);
h) of from 0 to 1 % by mass of chromium (Cr);
i) of from 0 to 1 % by mass of zirconium (Zr);
j) of from 0 to 0.5 % by mass of vanadium (V);
k) of from 0 to 0.06 % by mass of copper (Cu);
l) of from 0 to 1 % by mass of silicon (Si);
m) of from 0 to 1 % by mass of nickel (Ni);
n) of from 0 to 0.5 % by mass of cobalt (Co);

wherein the aluminium alloy further comprises inevitable impurities;
with the balance being aluminium (Al);
each amount in relation to the total mass of the alloy composition, and wherein all compounds of the alloy add up to a total of 100 % by mass.

It has been found that the aluminium alloy of the first aspect has high tensile strength (Rₘ), high yield strength (R_{p0.2}) and good elongation (A). In particular, when the alloy is used in a method of extrusion or another wrought process, products made of the alloy according to the first aspect of the present disclosure have a high tensile strength, a high yield strength and good elongation.

In a preferred embodiment of the first aspect, the aluminium alloy is suitable for extrusion and/or wrought applications.

In another preferred embodiment, the inevitable impurities are present in an amount of less than 0.15 % by mass, or in an amount of less than 0.1 % by mass, or in an amount of less than 0.05 % by mass. This relates to the total amount of impurities as present in the alloy.

In another preferred embodiment, each individual impurity is present in an amount of less than 0.05 % by mass, or in an amount of less than 0.01 % by mass, or in an amount of less than 0.001 % by mass, or in an amount of less than 0.0001 % by mass. If more than one impurity is present, each impurity is termed as "individual impurity". The amount of each individual impurity is preferably less than the respective given amount, and the sum of the amounts of each individual impurity results in the total amount of impurities.

One of these individual impurities may be thallium (Ta), resulting in an amount of Ta of less than 0.05 % by mass, or in an amount of less than 0.01 % by mass, or in an amount of less than 0.001 % by mass, or in an amount of less than 0.0001 % by mass.

Another one of these individual impurities may be gallium (Ga), resulting in an amount of Ga of less than 0.05 % by mass, or in an amount of less than 0.01 % by mass, or in an amount of less than 0.001 % by mass, or in an amount of less than 0.0001 % by mass.

Still another one of these individual impurities may be indium (In), resulting in an amount of In of less than 0.05 % by mass, or in an amount of less than 0.01 % by mass, or in an amount of less than 0.001 % by mass, or in an amount of less than 0.0001 % by mass.

Other examples of individual impurities include cerium (Ce), hafnium (Hf), lanthanum (La), niobium (Nb), molybdenum (Mo), yttrium (Y), or phosphor (P).

As one of the essential elements, the aluminium alloy according to the first aspect of the present disclosure contains magnesium (Mg) as a main ingredient in an amount of from 6 to 12 % by mass.

In a preferred embodiment of the first aspect, Mg is present in an amount of from 6.5 to 12 % by mass. In another preferred embodiment of the first aspect, Mg is present in an amount of from 7 to 12 % by mass. In another preferred embodiment of the first aspect, Mg is present in an amount of from 7. to 12 % by mass. In another preferred embodiment of the first aspect, Mg is present in an amount of from 8 to 12 % by mass. In another preferred embodiment of the first aspect, Mg is present in an amount of from 8 to 11.5 % by mass.

In another preferred embodiment of the first aspect, Mg is present in an amount of from 6 to 10 % by mass. In another preferred embodiment of the first aspect, Mg is present in an amount of from 6.5 to 9.5 % by mass. In another preferred embodiment of the first aspect, Mg is present in an amount of from 7 to 9 % by mass. In another preferred embodiment of the first aspect, Mg is present in an amount of from 7.5 to 8.5 % by mass. In another preferred embodiment of the first aspect, Mg is present in an amount of from 8 to 8.5 % by mass.

In another preferred embodiment of the first aspect, Mg is present in an amount of from 8 to 12 % by mass. In another preferred embodiment of the first aspect, Mg is present in an amount of from 9 to 12 % by mass. In another preferred embodiment of the first aspect, Mg is present in an amount of from 9.5 to 12 % by mass. In another preferred embodiment of the first aspect, Mg is present in an amount of from 10 to 12 % by mass. In another preferred embodiment of the first aspect, Mg is present in an amount of from 11 to 12 % by mass. In another preferred embodiment of the first aspect, Mg is present in an amount of from 11 to 11.5 % by mass.

It is understood that Mg is added to provide the strength and elongation to the resultant aluminium alloy product through solid solution strengthening after extrusion. If Mg is present in an amount of less than 6 % by weight, the yield strength and elongation of the aluminium alloy products is reduced. On the other hand, when the Mg content exceeds 12 % by mass, the hot workability of the alloy billet or slab is rapidly lowered. This feature in turn, makes it substantially difficult to manufacture the aluminium alloy products, in particular by extrusion or other means of wrought administrations.

Another essential element in the composition of the aluminium alloy according to the first aspect of the present disclosure is titanium (Ti), present in an amount of from 0.01 to 0.4 % by mass in relation to the total mass of the aluminium alloy composition.

In a preferred embodiment, Ti is present in an amount of from 0.01 to 0.3 % by mass. In a further preferred embodiment, Ti is present in an amount of from 0.01 to 0.3 % by mass. In a further preferred embodiment, Ti is present in an amount of from 0.01 to 0.2 % by mass. In a further preferred embodiment, Ti is present in an amount of from 0.015 to 0.15 % by mass. In a further preferred embodiment, Ti is present in an amount of from 0.015 to 0.08 % by mass.

In another embodiment, Ti is present in an amount of 0.4 % by mass or less. In a preferred embodiment, Ti is present in an amount of 0.3 % by mass or less. In a further preferred embodiment, Ti is present in an amount of 0.2 % by mass or less. In a further preferred embodiment, Ti is present in an amount of 0.15 % by mass or less. In a further preferred embodiment, Ti is present in an amount of 0.1 % by mass or less. In a further preferred embodiment, Ti is present in an amount of 0.08 % by mass or less.

In another embodiment, Ti is present in an amount of 0.01 % by mass or more. In a preferred embodiment, Ti is present in an amount of 0.015 % by mass or more.

The aluminium alloy according to the first aspect of the present disclosure contains manganese (Mn) at an amount of 2.5 % by mass or less. In a preferred embodiment, Mn is present in an amount 1.5 % by mass or less. In a further preferred embodiment, Mn is present in an amount of 1 % by mass or less. In a further preferred embodiment, Mn is present in an amount of 0.5 % by mass or less. In a further preferred embodiment, Mn is present in an amount of 0.1 % by mass or less. In a further preferred embodiment, Mn is present in an amount of 0.05 % by mass or less. In a further preferred embodiment, Mn is present in an amount of 0.01 % by mass or less. In a further preferred embodiment, Mn is present in an amount of 0.005 % by mass or less. In a further preferred embodiment, Mn is present in an amount of 0.0001 % by mass or more. In a further preferred embodiment, Mn is present in an amount of 0.0005 % by mass or more.

Also, the aluminium alloy according to the first aspect of the present disclosure contains iron (Fe) at an amount of 0.15 % by mass or less. In a preferred embodiment, Fe is present in an amount 0.1 % by mass or less. In a further preferred embodiment, Fe is present in an amount of 0.09 % by mass or less. In a further preferred embodiment, Fe is present in an amount of 0.08 % by mass or less. In a further preferred embodiment, Fe is present in an amount of 0.01 % by mass or more. In a further preferred embodiment, Fe is present in an amount of 0.05 % by mass or more.

Another element in the aluminium alloy according to the first aspect of the present disclosure is beryllium (Be), present in an amount of from 0.002 to 0.2 % by mass in relation to the total mass of the aluminium alloy composition. In a preferred embodiment, Be is present in an amount of from 0.002 to 0.15 % by mass. In a preferred embodiment, Be is present in an amount of from 0.003 to 0.1 % by mass. In a further preferred embodiment, Be is present in an amount of from 0.004 to 0.05 % by mass. In a further preferred embodiment, Be is present in an amount of from 0.005 to 0.02 % by mass. In a further preferred embodiment, Be is present in an amount of from 0.002 % by mass or more. In a further preferred embodiment, Be is present in an amount of from 0.003 % by mass or more. In a further preferred embodiment, Be is present in an amount of from 0.004 % by mass or more. In a further preferred embodiment, Be is present in an amount of from 0.005 % by mass or more. In a further preferred embodiment, Be is present in an amount of from 0.01 % by mass or more. In a further preferred embodiment, Be is present in an amount of from 0.015 % by mass or more. In a further preferred embodiment, Be is present in an amount of from 0.15 % by mass or less. In a further preferred embodiment, Be is present in an amount of from 0.1 % by mass or less. In a further preferred embodiment, Be is present in an amount of from 0.05 % by mass or less. In a further preferred embodiment, Be is present in an amount of from 0.02 % by mass or less.

It is understood that Be is added to prevent oxidation of the molten metal at the time of melting and casting of the alloy. Be also prevents loss of Mg and superficial change of colour which usually results from oxidation of the slab during melting, extrusion and/or heat treatment. When the Be content is less than 0.002 % by mass, Be is unable to effective prevent oxidation of the alloy composition. On the other hand, a Be content of more than 0.2 % by mass results in toxicity which substantially impairs the manufacturing process.

In a preferred embodiment of the aluminium alloy according to the first aspect of the present disclosure, boron (B) is present in an amount of from 0.001 to 0.1 % by mass. In a further preferred embodiment, B is present in an amount of from 0.002 to 0.08 % by mass. In a further preferred embodiment, B is present in an amount of from 0.002 to 0.06 % by mass. In a further preferred embodiment, B is present in an amount of from 0.002 to 0.04 % by mass. In a further preferred embodiment, B is present in an amount of from 0.003 to 0.02 % by mass. In a further preferred embodiment, B is present in an amount of from 0.003 to 0.016 % by mass. In a further preferred embodiment, B is present in an amount of 0.002 % by mass or more. In a further preferred embodiment, B is present in an amount of 0.0025 % by mass or more. In a further preferred embodiment, B is present in an amount of 0.003 % by mass or more. In a further preferred embodiment, B is present in an amount of 0.08 % by mass or less. In a further preferred embodiment, B is present in an amount of 0.06 % by mass or less. In a further preferred embodiment, B is present in an amount of 0.04 % by mass or less. In a further preferred embodiment, B is present in an amount of 0.02 % by mass or less. In a further preferred embodiment, B is present in an amount of 0.016 % by mass or less.

In a preferred embodiment of the present disclosure, Ti and B are added to the aluminium alloy melt together, further preferably in bars containing Ti and B in a ration of Ti:B of about 5:1, about 3:1 or about 1,6:1,4, such as TiBloy^{®}. However, the ration of Ti and B in the final alloy may differ from the ratio of Ti and B when added to the melt. Without being bound to said theory, it is assumed that some of the B is removed when removing the dross from the melt. Said dross is removed as it contains agglomerated impurities which are not desired in the final alloy. It is furthermore assumed that B is enriched in said dross, in particular in relation to Ti, due to the low specific weight of B. As such, it is preferred that the ration of Ti:B in the final alloy is in the range of from 3:1 to 10:1, preferably 5:1 to 10:1.

Ti and B form TiB₂ in the molten alloy. Hence, TiB₂ acts as nucleating agent during solidification of the molten aluminium alloy and hence refines the alloy. Thus, both strength and ductility are increased.

Another element in the aluminium alloy according to the first aspect of the present disclosure is silicon (Si), present in an amount of from 0 to 1 % by mass in relation to the total mass of the aluminium alloy composition. In a preferred embodiment, Si is present in an amount of 0.6 % by mass or less. In a further preferred embodiment, Si is present in an amount of 0.4 % by mass or less. In a further preferred embodiment, Si is present in an amount of 0.3 % by mass or less. In a further preferred embodiment, Si is present in an amount of 0.15 % by mass or less. In a further preferred embodiment, Si is present in an amount of 0.1 % by mass or less. In another preferred embodiment, Si is present in an amount of 0.001 % by mass or more. In a further preferred embodiment, Si is present in an amount of 0.005 % by mass or more.

It is understood that Si is added to the aluminium alloys to enhance the strength of the aluminium alloy by solid solution strengthening. Furthermore, Si binds excess Mg thus preventing the precipitation of coarse particles of Mg. Upon crystallization, Si and Mg form Mg₂Si intermetallic compounds, which increases the strength through precipitation hardening. On the other hand, elongation/ductility is reduced. Therefore, Si may only be added to alloys having a high elongation, such as 50 % or more, to further improve its strength. In other words, Si is added to alloy having an elongation of 50 % or more.

Another element in the aluminium alloy according to the first aspect of the present disclosure is copper (Cu), present in an amount of from 0 to 0.06 % by mass in relation to the total mass of the aluminium alloy composition. In a preferred embodiment, Cu is present in an amount of 0.05 % by mass or less. In a further preferred embodiment, Cu is present in an amount of 0.03 % by mass or less. In a further preferred embodiment, Cu is present in an amount of 0.02 % by mass or less. In a further preferred embodiment, Cu is present in an amount of 0.01 % by mass or less. In a further preferred embodiment, Cu is present in an amount of 0.005 % by mass or less. In another preferred embodiment, Cu is present in an amount of 0.001 % by mass or more. In a further preferred embodiment, Cu is present in an amount of 0.004 % by mass or more.

It is understood that Cu might only be added in an amount of up to 0.06 % by mass. If Cu is present in an amount of more than 0.06 % by mass, the aluminium alloy is susceptible to corrosion.

Another element in the aluminium alloy according to the first aspect of the present disclosure is zinc (Zn), present in an amount of from 0 to 5 % by mass in relation to the total mass of the aluminium alloy composition. In a preferred embodiment, Zn is present in an amount of 2.5 % by mass or less. In a further preferred embodiment, Zn is present in an amount of 1 % by mass or less. In a further preferred embodiment, Zn is present in an amount of 0.5 % by mass or less. In a further preferred embodiment, Zn is present in an amount of 0.1 % by mass or less. In a further preferred embodiment, Zn is present in an amount of 0.05 % by mass or less.

It is understood that Zn is added to the aluminium alloys to enhance the strength of the aluminium alloy by solid solution strengthening. Furthermore, Zn binds excess Mg forming MgZn₂ thus preventing the precipitation of coarse particles of Mg.

Another element in the aluminium alloy according to the first aspect of the present disclosure is chromium (Cr), present in an amount of from 0 to 1 % by mass in relation to the total mass of the aluminium alloy composition. In a preferred embodiment, Cr is present in an amount of 0.5 % by mass or less. In a further preferred embodiment, Cr is present in an amount of 0.2 % by mass or less. In a further preferred embodiment, Cr is present in an amount of 0.1 % by mass or less. In a further preferred embodiment, Cr is present in an amount of 0.05 % by mass or less. In a further preferred embodiment, Cr is present in an amount of 0.01 % by mass or less.

Another element in the aluminium alloy according to the first aspect of the present disclosure is zirconium (Zr), present in an amount of from 0 to 1 % by mass in relation to the total mass of the aluminium alloy composition. In a preferred embodiment, Zr is present in an amount of 0.5 % by mass or less. In a further preferred embodiment, Zr is present in an amount of 0.2 % by mass or less. In a further preferred embodiment, Zr is present in an amount of 0.1 % by mass or less. In a further preferred embodiment, Zr is present in an amount of 0.05 % by mass or less. In a further preferred embodiment, Zr is present in an amount of 0.05 % by mass or less.

Titanium, boron, manganese, zirconium, and chromium are added for grain refinement and to enhance the strength of the aluminium alloys. Even small amounts of these serve as nuclei during solidification of a molten aluminium alloy, so that it solidifies in many places at the same time, which results in a finer structure after extrusion and thus higher strength of aluminium alloy products.

Another element in the aluminium alloy according to the first aspect of the present disclosure is vanadium (V), present in an amount of from 0 to 0.5 % by mass in relation to the total mass of the aluminium alloy composition. In a preferred embodiment, V is present in an amount of 0.25 % by mass or less. In a further preferred embodiment, V is present in an amount of 0.15 % by mass or less. In a further preferred embodiment, V is present in an amount of 0.1 % by mass or less. In a further preferred embodiment, V is present in an amount of 0.05 % by mass or less. In a further preferred embodiment, V is present in an amount of 0.01 % by mass or less.

It is understood that V is added to the aluminium alloy composition in combination with Be to prevent oxidation of the molten metal at the time of melting and casting of the alloy.

Another element in the aluminium alloy according to the first aspect of the present disclosure is nickel (Ni), present in an amount of from 0 to 1 % by mass in relation to the total mass of the aluminium alloy composition. In a preferred embodiment, Ni is present in an amount of 0.5 % by mass or less. In a further preferred embodiment, Ni is present in an amount of 0.2 % by mass or less. In a further preferred embodiment, Ni is present in an amount of 0.1 % by mass or less. In a further preferred embodiment, Ni is present in an amount of 0.05 % by mass or less. In a further preferred embodiment, Ni is present in an amount of 0.01 % by mass or less.

Another element in the aluminium alloy according to the first aspect of the present disclosure is cobalt (Co), present in an amount of from 0 to 0.5 % by mass in relation to the total mass of the aluminium alloy composition. In a preferred embodiment, Co is present in an amount of 0.3 % by mass or less. In a further preferred embodiment, Co is present in an amount of 0.2 % by mass or less. In a further preferred embodiment, Co is present in an amount of 0.1 % by mass or less. In a further preferred embodiment, Co is present in an amount of 0.05 % by mass or less. In a further preferred embodiment, Co is present in an amount of 0.01 % by mass or less.

It is understood that both Ni and Co are added to the aluminium alloys to increase the temperature of recrystallization. This is of particular interest in the manufacture of aluminium alloy products by extrusion or other means of wrought applications because the alloy is stabilized at high temperatures. Furthermore, Ni and Co can bind excess Mg thus preventing the precipitation of coarse particles of Mg.

In another preferred embodiment, the aluminium alloy according to the first aspect of the present disclosure optionally comprises at least one element in an amount of from 0 to 0.5 % by mass in relation to the total mass of the aluminium alloy composition, wherein the at least one element is selected from the group consisting of Molybdenum (Mo), Hafnium (Hf), Calcium (Ca), Gallium (Ga), Scandium (Sc), Niobium (Nb), and Cerium (Ce). In another preferred embodiment, said at least one element is present in an amount of from 0 to 0.2 % by mass. In another preferred embodiment, the at least one element is present in an amount of from 0 to 0.1 % by mass. In another preferred embodiment, said at least one element is present in an amount of from 0 to 0.05 % by mass.

In one embodiment, the present disclosure relates to an aluminium alloy, comprising
a) of from 6 to 12 % by mass of magnesium (Mg);
b) of from 0.01 to 0.4 % by mass of titanium (Ti);
c) of from 0.002 to 0.08 % by mass of boron (B);
d) of from 0.002 to 0.1 % by mass of beryllium (Be);
e) of from 0 to 0.5 % by mass of manganese (Mn);
f) of from 0 to 0.1 % by mass of iron (Fe);
g) of from 0 to 2.5 % by mass of zinc (Zn);
h) of from 0 to 0.5 % by mass of chromium (Cr);
i) of from 0 to 0.5 % by mass of zirconium (Zr);
j) of from 0 to 0.25 % by mass of vanadium (V);
k) of from 0 to 0.05 % by mass of copper (Cu);
l) of from 0 to 0.6 % by mass of silicon (Si);
m) of from 0 to 0.5 % by mass of nickel (Ni);
n) of from 0 to 0.3 % by mass of cobalt (Co);

wherein the aluminium alloy further comprises inevitable impurities;
with the balance being aluminium (Al);
each amount in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 6.5 to 12 % by mass of magnesium (Mg);
b) of from 0.015 to 0.15 % by mass of titanium (Ti);
c) of from 0.003 to 0.03 % by mass of boron (B);
d) of from 0.003 to 0.1 % by mass of beryllium (Be);
e) of from 0 to 1 % by mass of manganese (Mn);
f) of from 0 to 0.1 % by mass of iron (Fe);
g) of from 0 to 2.5 % by mass of zinc (Zn);
h) of from 0 to 0.2 % by mass of chromium (Cr);
i) of from 0 to 0.2 % by mass of zirconium (Zr);
j) of from 0 to 0.1 % by mass of vanadium (V);
k) of from 0 to 0.05 % by mass of copper (Cu);
l) of from 0 to 0.5 % by mass of silicon (Si);
m) of from 0 to 0.5 % by mass of nickel (Ni);
n) of from 0 to 0.3 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 6 to 10 % by mass of magnesium (Mg);
b) of from 0.01 to 0.2 % by mass of titanium (Ti);
c) of from 0.002 to 0.04 % by mass of boron (B);
d) of from 0.003 to 0.1 % by mass of beryllium (Be);
e) of from 0 to 1 % by mass of manganese (Mn);
f) of from 0 to 0.1 % by mass of iron (Fe);
g) of from 0 to 2.5 % by mass of zinc (Zn);
h) of from 0 to 0.2 % by mass of chromium (Cr);
i) of from 0 to 0.2 % by mass of zirconium (Zr);
j) of from 0 to 0.1 % by mass of vanadium (V);
k) of from 0 to 0.05 % by mass of copper (Cu);
l) of from 0 to 0.6 % by mass of silicon (Si);
m) of from 0 to 0.1 % by mass of nickel (Ni);
n) of from 0 to 0.1 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7 to 9 % by mass of magnesium (Mg);
b) of from 0.015 to 0.15 % by mass of titanium (Ti);
c) of from 0.003 to 0.03 % by mass of boron (B);
d) of from 0.004 to 0.05 % by mass of beryllium (Be);
e) of from 0 to 0.1 % by mass of manganese (Mn);
f) of from 0 to 0.1 % by mass of iron (Fe);
g) of from 0 to 1 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.05 % by mass of copper (Cu);
l) of from 0 to 0.4 % by mass of silicon (Si);
m) of from 0 to 0.5 % by mass of nickel (Ni);
n) of from 0 to 0.3 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7.5 to 8.5 % by mass of magnesium (Mg);
b) of from 0.015 to 0.15 % by mass of titanium (Ti);
c) of from 0.003 to 0.03 % by mass of boron (B);
d) of from 0.004 to 0.05 % by mass of beryllium (Be);
e) of from 0 to 0.1 % by mass of manganese (Mn);
f) of from 0 to 0.1 % by mass of iron (Fe);
g) of from 0 to 1 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.05 % by mass of copper (Cu);
l) of from 0 to 0.4 % by mass of silicon (Si);
m) of from 0 to 0.5 % by mass of nickel (Ni);
n) of from 0 to 0.3 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7.5 to 8.5 % by mass of magnesium (Mg);
b) of from 0.015 to 0.1 % by mass of titanium (Ti);
c) of from 0.003 to 0.03 % by mass of boron (B);
d) of from 0.004 to 0.05 % by mass of beryllium (Be);
e) of from 0 to 0.05 % by mass of manganese (Mn);
f) of from 0.01 to 0.1 % by mass of iron (Fe);
g) of from 0 to 0.5 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.03 % by mass of copper (Cu);
l) of from 0 to 0.3 % by mass of silicon (Si);
m) of from 0 to 0.2 % by mass of nickel (Ni);
n) of from 0 to 0.1 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7.5 to 8.5 % by mass of magnesium (Mg);
b) of from 0.015 to 0.1 % by mass of titanium (Ti);
c) of from 0.003 to 0.03 % by mass of boron (B);
d) of from 0.005 to 0.02 % by mass of beryllium (Be);
e) of from 0 to 0.05 % by mass of manganese (Mn);
f) of from 0.01 to 0.1 % by mass of iron (Fe);
g) of from 0 to 0.1 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.03 % by mass of copper (Cu);
I) of from 0 to 0.15 % by mass of silicon (Si);
m) of from 0 to 0.1 % by mass of nickel (Ni);
n) of from 0 to 0.05 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7.5 to 8.5 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.03 % by mass of copper (Cu);
l) of from 0 to 0.15 % by mass of silicon (Si);
m) of from 0 to 0.05 % by mass of nickel (Ni);
n) of from 0 to 0.05 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7.5 to 8.5 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 8 to 8.5 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 8 to 12 % by mass of magnesium (Mg);
b) of from 0.015 to 0.15 % by mass of titanium (Ti);
c) of from 0.003 to 0.03 % by mass of boron (B);
d) of from 0.004 to 0.05 % by mass of beryllium (Be);
e) of from 0 to 0.1 % by mass of manganese (Mn);
f) of from 0 to 0.1 % by mass of iron (Fe);
g) of from 0 to 1 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.05 % by mass of copper (Cu);
l) of from 0 to 0.4 % by mass of silicon (Si);
m) of from 0 to 0.5 % by mass of nickel (Ni);
n) of from 0 to 0.3 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 8 to 12 % by mass of magnesium (Mg);
b) of from 0.015 to 0.1 % by mass of titanium (Ti);
c) of from 0.003 to 0.03 % by mass of boron (B);
d) of from 0.004 to 0.05 % by mass of beryllium (Be);
e) of from 0 to 0.05 % by mass of manganese (Mn);
f) of from 0.01 to 0.1 % by mass of iron (Fe);
g) of from 0 to 0.5 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.03 % by mass of copper (Cu);
l) of from 0 to 0.3 % by mass of silicon (Si);
m) of from 0 to 0.2 % by mass of nickel (Ni);
n) of from 0 to 0.1 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 8 to 12 % by mass of magnesium (Mg);
b) of from 0.015 to 0.1 % by mass of titanium (Ti);
c) of from 0.003 to 0.03 % by mass of boron (B);
d) of from 0.005 to 0.02 % by mass of beryllium (Be);
e) of from 0 to 0.05 % by mass of manganese (Mn);
f) of from 0.01 to 0.1 % by mass of iron (Fe);
g) of from 0 to 0.1 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.03 % by mass of copper (Cu);
l) of from 0 to 0.15 % by mass of silicon (Si);
m) of from 0 to 0.1 % by mass of nickel (Ni);
n) of from 0 to 0.05 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 9 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.05 % by mass of chromium (Cr);
i) of from 0 to 0.05 % by mass of zirconium (Zr);
j) of from 0 to 0.05 % by mass of vanadium (V);
k) of from 0 to 0.03 % by mass of copper (Cu);
l) of from 0 to 0.15 % by mass of silicon (Si);
m) of from 0 to 0.05 % by mass of nickel (Ni);
n) of from 0 to 0.05 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 9.5 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 9.5 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 10 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 11 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 11 to 11.5 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 6.5 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 7.5 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 8 to 12 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

In one embodiment, the present disclosure relates to an aluminium alloy, comprising
a) of from 8 to 11.5 % by mass of magnesium (Mg);
b) of from 0.015 to 0.08 % by mass of titanium (Ti);
c) of from 0.003 to 0.016 % by mass of boron (B);
d) of from 0.005 to 0.02 % by mass of beryllium (Be);
e) of from 0 to 0.01 % by mass of manganese (Mn);
f) of from 0.05 to 0.09 % by mass of iron (Fe);
g) of from 0 to 0.05 % by mass of zinc (Zn);
h) of from 0 to 0.01 % by mass of chromium (Cr);
i) of from 0 to 0.01 % by mass of zirconium (Zr);
j) of from 0 to 0.01 % by mass of vanadium (V);
k) of from 0 to 0.01 % by mass of copper (Cu);
l) of from 0 to 0.1 % by mass of silicon (Si);
m) of from 0 to 0.01 % by mass of nickel (Ni);
n) of from 0 to 0.01 % by mass of cobalt (Co);
o) wherein the aluminium alloy further comprises inevitable impurities;
p) with the balance being aluminium (Al);
each in relation to the total mass of the alloy composition, and wherein all compounds of the alloy add up to a total of 100 % by mass; wherein the aluminium alloy comprises inevitable impurities, preferably wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.

Aluminium alloys of the first aspect of the present disclosure, i.e. the aluminium alloys of the above compositions, have excellent mechanical properties in terms of high strength, in particular high yield and/or high tensile strengths, and high elongation at the same time. Furthermore, the aluminium alloys according to the first aspect are resistant to corrosion. Additionally, the aluminium alloys according to the first aspect are anodizable, i.e. the aluminium alloys are suitable for anodising.

### Aluminium alloy product

In a second aspect, the present disclosure relates to an aluminium alloy product comprising or consisting of an aluminium alloy according to the first aspect as disclosed above.

According to one embodiment, the aluminium product according to the second aspect of the present disclosure is an aluminium profile.

Aluminium profiles find broad application due to their low weight and ideal formability during manufacture. The majority of profiles have longitudinal slots in which sliding blocks can be inserted or swivelled in. These sliding blocks have a threaded hole and can be moved within the groove.

In addition to sliding blocks, other accessories can be inserted in the aforementioned longitudinal slots: Materials such as acrylic glass, double-webbed sheets, polycarbonate sheets, and the like. Furthermore, the longitudinal slots can be used to accommodate seals, adjustable feet and sliding elements.

According to one embodiment, the aluminium product according to the second aspect of the present disclosure is an extruded aluminium profile.

According to a preferred embodiment, the extruded aluminium profile is an extruded aluminium hollow profile. According to a further preferred embodiment, the extruded aluminium profile is an extruded aluminium massive profile.

In a preferred embodiment, the extruded aluminium profile has least parts which have a thickness in the range of from 1 to 15 mm, preferably 1 to 10 mm, preferably from 2 to 8 mm, preferably from 2 to 6 mm; or 2 to 5 mm, preferably 2.5 to 4 mm.

It is understood that the parts having the thickness in the range as described above is the smallest diameter of the extruded aluminium hollow profile or of the extruded massive aluminium profile.

In another embodiment, the thickness refers to the thickness of the aluminium alloy part of the extruded aluminium profile. In one embodiment, the thickness of an extruded aluminium hollow profile is the thickness of the walls of the profile.

In one embodiment, the aluminium alloy of the extruded aluminium profile has a tensile strength Rₘ of at least 260 MPa. In a preferred embodiment, the aluminium alloy of the extruded aluminium profile has a tensile strength Rₘ of at least 280 MPa. In a preferred embodiment, the aluminium alloy of the extruded aluminium profile has a tensile strength Rₘ of at least 300 MPa. In a further preferred embodiment, the aluminium alloy of the extruded aluminium profile has a tensile strength Rₘ of at least 320 MPa. In a further preferred embodiment, the aluminium alloy of the extruded aluminium profile has a tensile strength Rₘ of at least 350 MPa.

In one embodiment, the aluminium alloy of the extruded aluminium profile has a yield strength R_{p0.2} of at least 100 MPa. In a preferred embodiment, the aluminium alloy of the extruded aluminium profile has a yield strength R_{p0.2} of at least 140 MPa. In a further preferred embodiment, the aluminium alloy of the extruded aluminium profile has a yield strength R_{p0.2} of at least 180 MPa. In a further preferred embodiment, the aluminium alloy of the extruded aluminium profile has a yield strength R_{p0.2} of at least 190 MPa.

In one embodiment, the aluminium alloy of the extruded aluminium profile has an elongation A of at least 15 %. In a preferred embodiment, the aluminium alloy of the extruded aluminium profile has an elongation A of at least 20 %. In a further preferred embodiment, the aluminium alloy of the extruded aluminium profile has an elongation A of at least 25 %. In a further preferred embodiment, the aluminium alloy of the extruded aluminium profile has an elongation A of at least 30 %. In a further preferred embodiment, the aluminium alloy of the extruded aluminium profile has an elongation A of at least 35 %. In a further preferred embodiment, the aluminium alloy of the extruded aluminium profile has an elongation A of at least 40 %. In a further preferred embodiment, the aluminium alloy of the extruded aluminium profile has an elongation A of at least 45 %.

In one embodiment, the aluminium alloy of the extruded aluminium profile has a ratio X between the elongation A and the tensile strength Rₘ calculated as $X = \frac{elongation A \left[%\right]}{tensile strength {R}_{m} \left[MPa\right]}$

In one preferred embodiment, the aluminium alloy of the extruded aluminium product has a ratio X of at least 0.05 %/MPa. In a further preferred embodiment, the aluminium alloy of the extruded aluminium product has a ratio X of at least 0.07 %/MPa. In a further preferred embodiment, the aluminium alloy of the extruded aluminium product has a ratio X of at least 0.09 %/MPa. In a further preferred embodiment, the aluminium alloy of the extruded aluminium product has a ratio X of at least 0.11 %/MPa. In a further preferred embodiment, the aluminium alloy of the extruded aluminium product has a ratio X of at least 0.13 %/MPa. In a further preferred embodiment, the aluminium alloy of the extruded aluminium product has a ratio X of at least 0.15 %/MPa. In a further preferred embodiment, the aluminium alloy of the extruded aluminium product has a ratio X of at least 0.17 %/MPa.

In a further preferred embodiment of the second aspect of the disclosure, the aluminium product comprise a surface finishing. According to a further preferred embodiment of the second aspect of the disclosure, the aluminium product comprise a surface finishing which is an anodization. According to a further preferred embodiment of the second aspect of the disclosure, the aluminium product comprise a surface finishing which is a hard-anodization.

The shape of the aluminium alloy product according to the second aspect of the present disclosure is not particularly limited. According to a preferred embodiment, the cross-section of the aluminium products according to the second aspect of the present disclosure is rectangular. According to a further preferred embodiment, the cross-section of the aluminium products according to the second aspect of the present disclosure is a square. According to a further preferred embodiment, the cross-section of the aluminium products according to the second aspect of the present disclosure is circular. According to a further preferred embodiment, the cross-section of the aluminium products according to the second aspect of the present disclosure is elliptical. Optionally, the cross-section further contains massive or hollow parts extending from the rectangular, square, circular or elliptical cross-section.

The aluminium alloy products can advantageously be used in the manufacture of cars. In particular, the aluminium alloy products according to the second aspect of the present disclosure provide for advantageous properties when used in the construction of the front of a car, e.g., as longitudinal beam, or in the side impact protection in doors. Furthermore, the aluminium alloy products according to the second aspect of the present disclosure provide for advantageous properties in aluminium lightweight constructions.

### Method of manufacturing of an aluminium alloy

A third aspect of the present disclosure relates to a method for the manufacture of an aluminium alloy according to the first aspect as disclosed above, comprising the steps of
a) Providing a raw aluminium;
b) Heating the raw aluminium to a temperature in the range of from 650 to 850 °C, preferably from 750 to 800 °C;
c) Adding Mg and Be to result in a raw alloy;
d) Optionally degassing the raw alloy;
e) Adding Ti and B to the optionally degassed raw alloy to prepare the aluminium alloy; and
f) Casting the aluminium alloy to prepare an aluminium billet.

The raw aluminium is preferably provided having a low amount of impurities, preferably having a level of impurity of 0.3 % by mass or less in relation to the total mass of the raw aluminium. The raw aluminium is then heated in a furnace to a temperature melting the aluminium, but not heating the aluminium too high, in particular not above 900 °C, in order to avoid the formation of excess oxidation products. It is therefore preferred to heat the raw aluminium to a temperature in the range of from 650 to 850 °C. In a further preferred embodiment, the raw aluminium is heated to a temperature in the range of from 750 to 700 °C. In a further preferred embodiment, the raw aluminium is heated to a temperature in the range of from 750 to 770 °C. Prior to the addition of the raw aluminium to the furnace, the furnace may be pre-heated, preferably to a temperature in the range of from 400 to 900 °C.

Once the raw aluminium is melted, Mg and Be are added. As these metals are added in solid form, the temperature of the melt will drop. It is therefore preferred to re-heat the aluminium melt to a previously defined temperature or temperature range, or to maintain the previously defined temperature or temperature range during addition of the metals. Further optional elements, such as Mn, Fe, Cu, Zn or Si, may be added during this step.

The resulting raw aluminium alloy may then optionally be degassed using usual measures. In a preferred embodiment, the degassing may be supported by argon gas as purging gas.

After the addition of the above listed elements, and the optional degassing step, Ti and optionally B are added in a final step. In this step, also the further elements of the aluminium alloy can be added. In a preferred embodiment, manganese, iron, zinc, chromium, zirconium, vanadium, copper, silicon, nickel, and/or cobalt are added.

Furthermore, the raw aluminium alloy is refined.

The final aluminium alloy melt may then be cast, e.g., to billets for further or later processing, such as in the method of the fourth aspect or it may be directly used in step g) of the fourth aspect.

The aluminium alloy according to the first aspect of the present disclosure may be used in any known casting method, and the casting method is not limited by the aluminium of the present application. In particular, it may be used in any known casting method used for standard AlMg10 aluminium alloys. The liquid aluminium alloy may be cast into a mold. After cooling the mold, it may be removed, providing a billet comprising the aluminium alloy according to the first aspect of the present disclosure. The billet may then optionally be further processed in a usual and known manner.

In a preferred embodiment of the third aspect, the casting is selected from the group consisting of sand casting, plaster mold casting, shell casting, lost-wax casting, evaporative-pattern casting (e.g., lost foam casting or full-mold casting), permanent mold casting, die casting (preferably pressure die casting), semi-solid metal casting, centrifugal casting, and continuous casting.

According to a preferred embodiment of the third aspect, the aluminium billet may by a massive aluminium billet. According to another preferred embodiment of the third aspect, the aluminium billet may by a hollow aluminium billet.

In a further preferred embodiment of the third aspect, the liquid aluminium alloy and/or the aluminium billet is characterized by low or no formation of dross (i.e. aluminium dross). Aluminium dross may occur upon exposition of liquid aluminium alloy and/or molten aluminium casting to air. A longer exposition to air promotes an enhanced formation of dross. In a preferred embodiment of the third aspect, liquid aluminium alloy and/or molten aluminium casting is characterized by low or no formation of dross over a long-term exposition to air (e.g., 8 hours). The formation of dross may be visible to the bare eye and/or detectable by any technical method applicable thereto (e.g., spectral analysis).

### Manufacture of aluminium alloy product

In a fourth aspect, the present disclosure relate to a method for the manufacture of an aluminium alloy product according to the second aspect as disclosed above, wherein the manufacture of the aluminium alloy product comprises the steps of
g) Preheating an aluminium billet of an aluminium alloy according to the first aspect as disclosed above, to a temperature in the range of from 400 °C to 450 °C, preferably in the range of from 420 °C to 440 °C to result in a preheated aluminium billet;
h) Inserting the preheated aluminium billet from step g) into an extrusion press;
i) Extruding the preheated aluminium billet to result an extruded aluminium profile.

The advantages of extrusion are in particular the possibilities of producing profiles even in complex shapes and from materials, i.e. as high strength aluminium alloys as described in the first aspect of the present disclosure, which are difficult to form.

In one embodiment of the fourth aspect of the present disclosure, the aluminium billet is an aluminium alloy according to the first aspect of the present disclosure as described above.

In one embodiment of the fourth aspect of the present disclosure, the aluminium billet comprises or consists of an aluminium alloy according to the first aspect of the present disclosure.

In one embodiment of the fourth aspect of the present disclosure, the aluminium billet is provided in step f) of the method according to the third aspect of the present disclosure. In other words, the method of the third aspect and the fourth aspect may be combined to one method of manufacture of an aluminium alloy product according to the second aspect of the present disclosure.

In one embodiment of the fourth aspect of the present disclosure, the aluminium billet is heated to result in a preheated aluminium billet. In a preferred embodiment of the fourth aspect, the aluminium billet is heated to a temperature in the range of from 400 °C to 450 °C to result in a preheated aluminium billet. In a further preferred embodiment of the fourth aspect, the aluminium billet is heated to a temperature in the range of from 420 °C to 440 °C to result in a preheated aluminium billet.

According to one embodiment, the preheated aluminium billet described above is inserted into an extrusion press. In a preferred embodiment, the temperature of the aluminium billet is in the range of from 400 °C to 450 °C when it is inserted into the extrusion press. In a preferred embodiment, the temperature of the aluminium billet is in the range of from 420 °C to 440 °C when it is inserted into the extrusion press.

The extrusion press is not particularly limited. The extrusion press may be any extrusion press suitable for cold extrusion or warm extrusion or friction extrusion, preferably warm extrusion. It is understood that the extrusion press must be capable of carrying out an extrusion process as described in the following:
In one embodiment of the fourth aspect, extruding the preheated aluminium billet in the extrusion press results an extruded aluminium profile. The terms "extrusion", "extrusion process" and "extruding" as used herein are interchangeable.

According to a preferred embodiment of the fourth aspect, extruding is a direct extrusion. According to a further preferred embodiment, the preheated aluminium billet is placed in a heavy walled container within the extrusion press and the billet is pushed through a die by a ram or screw to result in an extruded aluminium profile according to the second aspect of the present disclosure.

In such direct extrusion process, a reusable block may be placed between the ram and the billet to keep them separated.

According to a preferred embodiment of the fourth aspect, extruding is an indirect extrusion. According to a further preferred embodiment, the preheated aluminium billet is placed in a heavy walled container within the extrusion press and the billet and container move together while the die is stationary. In other words, the die is held in place by a stem and the billet is moved and formed by the die.

In a further preferred embodiment of the fourth aspect, the force applied by the ram during extrusion does not exceed a maximum force of 20,000 kN. In a further preferred embodiment, extruding the preheated aluminium billet to result an extruded aluminium profile is carried out at a maximum force in the range of from 5,000 to 15,000 kN. In a further preferred embodiment, extruding the preheated aluminium billet to result an extruded aluminium profile is carried out at a maximum force in the range of from 7,000 to 12,000 kN. In a further preferred embodiment, extruding the preheated aluminium billet to result an extruded aluminium profile is carried out at a maximum force in the range of from 8,000 to 10,000 kN. In a further preferred embodiment, extruding the preheated aluminium billet to result an extruded aluminium profile is carried out at a maximum force of about 9,000 kN.

Neither the ram or screw nor the die of the extrusion press are particularly limited. The ram may be driven hydraulically. Suitable shapes of the die are known in the art.

According to one preferred embodiment of the fourth aspect of the present disclosure, the die is a spider die, porthole die or bridge die. Said designs of die are suitable for forming internal cavities in extrusion, i.e., aluminium hollow profiles, when a solid aluminium billet is used in the extrusion process. All of these types of dies incorporate a mandrel in the die and have "legs" that hold the mandrel in place. During extrusion, the metal divides, flows around the legs and then merges again.

According to a further preferred embodiment, the ram and/or the reusable block may have a mandrel. Said designs of the ram is suitable for forming internal cavities in extrusion, i.e., aluminium hollow profiles, when a hollow or massive aluminium billet is used in the extrusion process. If a massive aluminium billet is used, the massive aluminium billet must be pierced by the mandrel prior to extrusion.

According to a further preferred embodiment of the fourth aspect, the extruded aluminium profile is not subjected to a heat treatment after step i).

According to a further preferred embodiment of the fourth aspect, the extruded aluminium profile is heat treated after step i) by heating the extruded aluminium profile at a temperature of at least 380 °C, or at least 400 °C, or at least 430 °C, or at least 450 °C.

According to a further preferred embodiment of the fourth aspect, the extruded aluminium profile is heat treated after step i) for a period of less than 1 hour, or less than 3 hours, or less than 5 hours, or less than 8 hours, or less than 12 hours, or less than 18 hours, or less than 24 hours, preferably less than 12 hours, or preferably less than 18 hours, or for a period of at least 10 minutes, or at least 1 hour, or at least 3 hours, or at least 8 hours, or at least 12 hours, or at least 24 hours, and then cooled in air at ambient temperature.

Said heat treatment step may optionally be applied.

It is understood that heat treatment is applied to the aluminium alloy products to refine the grain structure. In particular, a heat treatment may be applied if the aluminium product comprises or consists of an aluminium alloy comprising 9 % by mass or more of Mg. A heat treatment may not be applied if the aluminium product comprises or consists of an aluminium alloy comprising less than 9 % by mass of Mg.

According to a preferred embodiment of the fourth aspect, the extruded aluminium profile comprising or consisting of an aluminium alloy comprising 9 % by mass or more of Mg is heat treated as described above. According to a further preferred embodiment of the fourth aspect, the extruded aluminium profile comprising or consisting of an aluminium alloy comprising 10 % by mass or more of Mg is heat treated as described above. According to a preferred embodiment of the fourth aspect, the extruded aluminium profile comprising or consisting of an aluminium alloy comprising 11 % by mass or more of Mg is heat treated as described above. According to a further preferred embodiment of the fourth aspect, the extruded aluminium profile comprising or consisting of an aluminium alloy comprising of from 9 to 14 % by mass of Mg is heat treated as described above. According to a further preferred embodiment of the fourth aspect, the extruded aluminium profile comprising or consisting of an aluminium alloy comprising of from 10 to 14 % by mass of Mg is heat treated as described above. According to a further preferred embodiment of the fourth aspect, the extruded aluminium profile comprising or consisting of an aluminium alloy comprising of from 11 to 14 % by mass of Mg is heat treated as described above.

According to a further preferred embodiment of the fourth aspect, the extruded aluminium profile comprising or consisting of an aluminium alloy comprising less than 9 % by mass of Mg is not heat treated. According to a further preferred embodiment of the fourth aspect, the extruded aluminium profile comprising or consisting of an aluminium alloy comprising of from 6 to 9 % by mass of Mg is not heat treated. According to a further preferred embodiment of the fourth aspect, the extruded aluminium profile comprising or consisting of an aluminium alloy comprising of from 6 to 8 % by mass of Mg is not heat treated.

According to a further preferred embodiment of the fourth aspect of the present disclosure, the extruded aluminium profile is optionally subjected to a treatment for surface finishing. According to a further preferred embodiment of the fourth aspect of the present disclosure, the extruded aluminium profile is optionally subjected to a treatment for surface finishing wherein the surface finishing is an anodization, with and without colours. According to a further preferred embodiment of the fourth aspect of the present disclosure, the extruded aluminium profile is optionally subjected to a treatment for surface finishing wherein the surface finishing is a hard-anodization.

### Aluminium alloy prepared by method of fourth aspect

In a fifth aspect, the present disclosure relates to an extruded aluminium profile prepared by a method according to the fourth aspect as disclosed above.

It is understood that the extruded aluminium profile according to the fifth aspect of the present disclosure has the same properties as the aluminium alloy product of the second aspect as described above.

### Use of aluminium alloy in extrusion or other wrought application

In a sixth aspect, the present disclosure relates to the use of an aluminium alloy according to the first aspect disclosed herein in an extrusion process or a wrought process.

According to a preferred embodiment of the sixths aspect, the extrusion is an indirect extrusion. According to a further preferred embodiment of the sixths aspect, the extrusion is a direct extrusion.

According to a further preferred embodiment of the sixths aspect, the wrought process is forging. According to a further preferred embodiment of the sixths aspect, the wrought process is semi-solid shaping.

### Definitions

The present invention as illustratively described in the following may suitably be practiced in the absence of any element or elements, limitation or limitations, not specifically disclosed herein.

The present invention will be described with respect to particular embodiments and with reference to certain figures but the invention is not limited thereto but only by the claims. Terms as set forth hereinafter are generally to be understood in their common sense unless indicated otherwise.

Where the term "comprising" is used in the present description and claims, it does not exclude other elements. For the purposes of the present invention, the term "consisting of" is considered to be a preferred embodiment of the term "comprising". If a group is defined to comprise at least a certain number of embodiments herein, this is also to be understood to disclose a group, which preferably consists only of these embodiments. Furthermore, if a composition is defined using the term "comprising", it may additionally comprise other elements not explicitly listed, however, not further amounts of an element listed. As such, if, e.g., an aluminium alloy comprises Mg in an amount of 12 % by mass, said aluminium alloy may comprise elements other than Mg, however, not additional amounts of Mg, thereby exceeding the amount of 12 % by mass.

The term "about" in conjunction with a numerical value refers to normal deviations of said numerical value. It is to be understood that the term "about" can mean a deviation of ± 10 %, preferably ± 5 %, more preferably ± 2.5 % of said numeric value as indicated.

Where an indefinite or definite article is used when referring to a singular noun, e.g. "a", "an" or "the", this includes a plural of that noun unless something else is specifically stated.

Terms like "obtainable" or "definable" and "obtained" or "defined" are used interchangeably. This e.g. means that, unless the context clearly dictates otherwise, the term "obtained" does not mean to indicate that e.g. an embodiment must be obtained by e.g. the sequence of steps following the term "obtained" even though such a limited understanding is always included by the terms "obtained" or "defined" as a preferred embodiment.

As used herein, the terms "impurity" and "impurities" refer to and comprises elements in the alloy which are inevitably present due to, e.g., the manufacturing process of the alloy or the manufacturing process of the raw material(s). An impurity is not explicitly mentioned in the list of elements in the alloy, however, an element may turn from an impurity to an essential element in the alloy. If, e.g., an element is not mentioned in a more general definition of the composition of an alloy, it may be present as an impurity, and the same element may be mentioned as a compulsory compound in a more specific definition of the composition of the alloy.

The aluminium alloy according to the first aspect of the present disclosure is composed of different components. These components are explicitly listed in the composition of the alloy, or they are part of the impurities present in the alloy. In any case, if a component is defined as an amount in % by mass, the figure reflects the relative amount (as mass) in percent based on the total mass of the alloy composition.

As used herein, the terms "tensile strength" and "ultimate tensile strength" are used interchangeably. The tensile strength may be abbreviated as "Rₘ". Methods for determining the tensile strength are known to the skilled person. As used herein, the tensile strength Rₘ is the maximum stress that a material can withstand while being stretched or pulled before breaking.

As used herein, the terms "yield strength" and "yield tensile strength" are used interchangeably. The yield strength may be abbreviated as "R_{p0.2}". Methods for determining the yield strength are known to the skilled person. As used herein, the tensile strength is the stress corresponding to the yield point at which the material begins to deform plastically. The yield point is the point on a stress-strain curve that indicates the limit of elastic behaviour and the beginning of plastic behaviour. Below the yield point, a material will deform elastically and will return to its original shape when the applied stress is removed. Once the yield point is passed, some fraction of the deformation will be permanent and non-reversible and is referred to as plastic deformation.

As used herein, the term "elongation" abbreviated as "A" is the elongation at fracture and indicates the permanent elongation of a tensile specimen after fracture, in relation to the initial gauge length of the tensile specimen. In other words, the elongation A is the permanent change in the length ΔL of a specimen in a tensile test after fracture has occurred in relation to the initial gauge length L₀ of the specimen.

As used herein, the terms yield strength Rₘ, tensile strength R_{p0.2}, elongation A, and the ratio X refer to the aluminium alloy of the aluminium product. In other words, terms yield strength Rₘ, R_{p0.2}, elongation, and the ratio X are measured on the aluminium part of the aluminium product.

The yield strength Rₘ, tensile strength R_{p0.2}, elongation A of the aluminium alloys are determined in accordance with DIN 50125:2009 at 23 °C.

As used herein, the term "extrusion" is a process used to create objects of a fixed cross-sectional profile by pushing a preheated billet of an aluminium alloy according to the first aspect of the present disclosure through a die of the desired cross-section. Extrusion may be continuous. In continuous extrusion, a theoretically indefinitely long aluminium alloy product can be produced. Extrusion may be semi-continuous. In semi-continuous extrusion, many pieces of identical size can be produced.

As used herein, the terms "aluminium profile" and "extruded aluminium profile" are used interchangeably. The term "extruded" means that the aluminium profile has been manufactured by extrusion as described above.

The term "hollow" as used herein, means that at least part of the aluminium hollow profile is not massive but has a hollow cross-section. In other words, the aluminium hollow profile has a hole or an empty space inside. The hollow part is filled with air.

The term "massive" as used herein, means that at least part of the aluminium profile is not hollow but has a massive cross-section. In other words, there are no empty space inside the massive aluminium profile.

As used herein, the term "cross-section" means the shape exposed by making a straight cut through the aluminium product according to the second aspect of the present disclosure at right angles to the direction of extrusion. The cross-section is determined by the die and/or mandrel used in the manufacturing, e.g., extrusion, process.

The terms "wrought applications" and "wrought process" are used interchangeably. As used herein, the term wrought application means any process which involves the shaping of metal with a high degree of shaping. In other words, a wrought application is the beating of a piece of metal into a shape by tools. One example of wrought application is forging. Another example of wrought application is semi-solid shaping.

### Examples

### Example 1: Manufacture of aluminium alloys

All aluminium alloys were prepared in a resistance-heated crucible furnace (Nabertherm, model K40/12). For the preparation of a 50 kg of raw aluminium melt, the raw aluminium (with 0.15 % by mass or less of total impurities; obtained from Adial, Adriers, France) was added into the furnace over a period of 1 h to result in a molten raw aluminium.

The raw aluminium was heated to 720 to 750 °C and the respective amounts of Mg (from DEUMU Deutsche Erz- und Metall-Union GmbH, Germany, pure magnesium, at least 99.8 %) and Be (added as pellets of AlBe, containing 5 % by mass of Be, the remainder being Al, from Hoesch Metals, Niederzier, Germany) were added. After re-heating to 720 to 750 °C, the melt was de-gassed for 10 minutes with Argon gas as purging gas using an injection lance.

Then, at a temperature in the range of 650 to 750 °C, Ti and B are added as bars containing Ti and B in a ratio of 5:1 (added as pellets of AlTi5B1, containing 5 % by mass of Ti, 1 % by mass of B, the remainder being Al, from Foseco-Vesuvius, Germany). The bars are stirred into the liquid alloy, and immediately after mixing, the furnace is tilted and the liquid alloy is cast into a respective mold to provide an aluminium alloy billet.

**Table 1 Composition of aluminium alloy. All amounts are given in % by mass in relation to the total mass of the aluminium alloy. The balance to the compositions disclosed in Table 1 is aluminium.**

| No. | Mg | Ti | Be | B | Si | Fe | Mn | Cu | Impurities |
|---|---|---|---|---|---|---|---|---|---|
| 1 | 8.26 | 0.015 | 0.005 | 0,003 | 0.099 | 0.086 | 0.005 | 0.004 | 0.066 |
| 2 | 11.40 | 0.071 | 0.016 | 0,014 | 0.005 | 0.080 | 0.004 | 0.001 | 0.084 |

### Example 2: Manufacture of aluminium hollow profiles

The aluminium alloy billets No. 1 and No. 2 of example 1 were preheated to a temperature in the range of from 400 to 450 °C and placed into an extrusion press (from SMS group, Germany; maximum pressing force of 9000 kN) for direct extrusion.

The extrusion process results an aluminium hollow profile with 30 mm height (also referred to the narrow side S), 60 mm width (also referred to as the broad side B), and a wall thickness s of 3 mm as depicted in Figure 1.

### Example 3: Heat treatment

The aluminium hollow profiles of example 2 were investigated for the mechanical properties with and without heat treatment.

The aluminium hollow profiles were heated to a temperature of 450 °C for 4 h in a furnace and then cooled to room temperature.

### Example 4: Mechanical properties

For evaluation of the mechanical properties, dumbbell-shaped samples were cut out of the narrow side S and the broad side B of the aluminium hollow profiles according to examples 2 and 3.

Both the heat treated and not heat treated samples were subjected to tests determining the tensile strength (Rₘ), the yield strength (R_{p0.2}) and the elongation (A). The measuring length was 30 mm for all samples having a thickness of 3 mm. All test results are summarized in Table 2 below.

The samples were prepared and tested in accordance with DIN 50125:2009 at room temperature (23 °C).

**Table 2 Mechanical properties of alloys No. 1 and No. 2**

| **No.** | heat treated | Rₘ [MPa] | R_{p0.2} [MPa] | A [%] |
|---|---|---|---|---|
| **1** | No | 308.4 | 182.0 | 51.6 |
| | Yes | 269.4 | 103.2 | 47.7 |
| | | | | |
| **2** | No | 340.8 | 190.4 | 26.4 |
| | Yes | 368.4 | 187.2 | 48.9 |

It can be seen from the above test results that the samples of the extruded aluminium hollow profiles of alloys No. 1 and No. 2 show excellent mechanical properties, in particular in terms of yield strength Rₘ, tensile strength R_{p0.2}, and elongation A. In particular, the samples have both high yield strength and elongation at the same time; with and without heat treatment.

### Items

The present disclosure also pertains to the following numbered items:
1. An aluminium alloy comprising
   a) of from 6 to 12 % by mass of magnesium (Mg);
   b) of from 0.01 to 0.5 % by mass of titanium (Ti);
   c) of from 0.001 to 0.1 % by mass of boron (B);
   d) of from 0.002 to 0.2 % by mass of beryllium (Be);
   e) of from 0 to 2.5 % by mass of manganese (Mn);
   f) of from 0 to 0.2 % by mass of iron (Fe);
   g) of from 0 to 5 % by mass of zinc (Zn);
   h) of from 0 to 1 % by mass of chromium (Cr);
   i) of from 0 to 1 % by mass of zirconium (Zr);
   j) of from 0 to 0.5 % by mass of vanadium (V);
   k) of from 0 to 0.06 % by mass of copper (Cu);
   l) of from 0 to 1 % by mass of silicon (Si);
   m) of from 0 to 1 % by mass of nickel (Ni);
   n) of from 0 to 0.5 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
2. The aluminium alloy according to item 1, wherein the aluminium alloy is suitable for extrusion and/or other wrought applications.
3. The aluminium alloy according to any one of items 1 or 2, wherein the inevitable impurities are present in an amount of less than 0.15 % by mass, preferably in an amount of less than 0.1 % by mass, further preferably in an amount of less than 0.05 % by mass, and each individual impurity is present in an amount of less than 0.05 % by mass, preferably in an amount of less than 0.01 % by mass, further preferably in an amount of less than 0.001 % by mass.
4. The aluminium alloy according to any one of items 1 to 3, wherein Mg is present in an amount of from 6.5 to 12 % by mass, preferably in an amount of from 7 to 12 % by mass, preferably in an amount of from 7.5 to 12 % by mass, preferably in an amount of from 8 to 12 % by mass, preferably in an amount of from 8 to 11.5 % by mass.
5. The aluminium alloy according to any one of items 1 to 3, wherein Mg is present in an amount of from 6 to 10 % by mass, preferably in an amount of from 6.5 to 9.5 % by mass, preferably in an amount of from 7 to 9 % by mass, preferably in an amount of from 7.5 to 8.5 % by mass, preferably in an amount of from 8 to 8.5 % by mass.
6. The aluminium alloy according to any one of items 1 to 3, wherein Mg is present in an amount of from 8 to 12 % by mass, preferably in an amount of from 9 to 12 % by mass, preferably in an amount of from 9.5 to 12 % by mass, preferably in an amount of from 10 to 12 % by mass, preferably in an amount of from 11 to 12 % by mass, preferably in an amount of from 11 to 11.5 % by mass.
7. The aluminium alloy according to any one of claims 1 to 6, wherein Ti is present
   i) in an amount of from 0.01 to 0.4 % by mass, preferably in an amount of from 0.01 to 0.3 % by mass, preferably in an amount of from 0.01 to 0.2 % by mass, preferably in an amount of from 0.015 to 0.15 % by mass, preferably in an amount of from 0.015 to 0.1 % by mass; preferably in an amount of from 0.015 to 0.08 % by mass; and/or
   ii) in an amount of from 0.4 % by mass or less, preferably in an amount of 0.3 % by mass or less, preferably in an amount of 0.2 % by mass or less, preferably in an amount of 0.15 % by mass or less, preferably in an amount of 0.1 % by mass or less; preferably in an amount of 0.08 % by mass or less; and/or
   iii) in an amount of 0.01 % by mass or more, preferably in an amount of 0.015 % by mass or more.
8. The aluminium alloy according to any one of items 1 to 7, wherein Mn is present
   i) in an amount of 1.5 % by mass or less, preferably in an amount of 1 % by mass or less, preferably in an amount of 0.5 % by mass or less, preferably in an amount of 0.1 % by mass or less, preferably in an amount of 0.05 % by mass or less, preferably in an amount of 0.01 % by mass or less, preferably in an amount of 0.005 % by mass or less; and/or
   ii) in an amount of 0.0001 % by mass or more, preferably in an amount of 0.0005 % by mass or more.
9. The aluminium alloy according to any one of items 1 to 8, wherein Fe is present
   i) in an amount of 0.15 % by mass or less, preferably in an amount of 0.1 % by mass or less, preferably in an amount of 0.09 % by mass or less, preferably in an amount of 0.08 % by mass or less; and/or
   ii) in an amount of 0.01 % by mass or more, preferably in an amount of 0.05 % by mass or more.
10. The aluminium alloy according to any one of claims 1 to 9, wherein Be is present
   i) in an amount of from 0.002 to 0.15 % by mass, preferably in an amount of from 0.003 to 0.1 % by mass, preferably in an amount of from 0.004 to 0.05 % by mass, preferably in an amount of from 0.005 to 0.02 % by mass; and/or
   ii) in an amount of 0.002 % by mass or more, or in an amount of 0.003 % by mass or more, or in an amount of 0.004 % by mass or more, or in an amount of 0.005 % by mass or more, or in an amount of 0.015 % by mass or more; and/or
   iii) in an amount of 0.15 % by mass or less, or in an amount of 0.1 % by mass or less, or in an amount of 0.05 % by mass or less, or in an amount of 0.02 % by mass or less.
11. The aluminium alloy according to any one of items 1 to 10, wherein B is present
   i) in an amount of from 0.002 to 0.08 % by mass, preferably in an amount of from 0.002 to 0.06 % by mass, preferably in an amount of from 0.002 to 0.04 % by mass, preferably in an amount of from 0.003 to 0.02 % by mass, preferably in an amount of from 0.003 to 0.016 % by mass; and/or
   ii) in an amount of 0.002 % by mass or more, or in an amount of 0.0025 % by mass or more, or in an amount of 0.003 % by mass or more; and/or
   iii) in an amount of 0.08 % by mass or less, or in an amount of 0.06 % by mass or less, or in an amount of 0.04 % by mass or less, or in an amount of 0.02 % by mass or less, or in an amount of 0.016 % by mass or less.
12. The aluminium alloy according to any one of items 1 to 11, wherein Si is present
   i) in an amount of 0.6 % by mass or less, preferably in an amount of 0.4 % by mass or less, preferably in an amount of 0.3 % by mass or less, preferably in an amount of 0.15 % by mass or less, preferably in an amount of 0.1 % by mass or less; and/or
   ii) in an amount of 0.001 % by mass or more, preferably in an amount of 0.005 % by mass or more.
13. The aluminium alloy according to any one of items 1 to 12, wherein Cu is present
   i) in an amount of 0.05 % by mass or less, preferably in an amount of 0.03 % by mass or less, preferably in an amount of 0.02 % by mass or less, preferably in an amount of 0.01 % by mass or less, preferably in an amount of 0.005 % by mass or less; and/or
   ii) in an amount of 0.001 % by mass or more, or in an amount of 0.004 % by mass or more.
14. The aluminium alloy according to any one of items 1 to 13, wherein Zn is present in an amount of 2.5 % by mass or less, preferably in an amount of 1 % by mass or less, preferably in an amount of 0.5 % by mass or less, preferably in an amount of 0.1 % by mass or less, preferably in an amount of 0.05 % by mass or less.
15. The aluminium alloy according to any one of items 1 to 14, wherein Cr is present in an amount of 0.5 % by mass or less, preferably in an amount of 0.2 % by mass or less, preferably in an amount of 0.1 % by mass or less, preferably in an amount of 0.05 % by mass or less, preferably in an amount of 0.01 % by mass or less.
16. The aluminium alloy according to any one of items 1 to 15, wherein Zr is present in an amount of 0.5 % by mass or less, preferably in an amount of 0.2 % by mass or less, preferably in an amount of 0.1 % by mass or less, preferably in an amount of 0.05 % by mass or less, preferably in an amount of 0.01 % by mass or less.
17. The aluminium alloy according to any one of items 1 to 16, wherein V is present in an amount of 0.25 % by mass or less, preferably in an amount of 0.15 % by mass or less, preferably in an amount of 0.1 % by mass or less, preferably in an amount of 0.05 % by mass or less, preferably in an amount of 0.01 % by mass or less.
18. The aluminium alloy according to any one of items 1 to 17, wherein Ni is present in an amount of 0.5 % by mass or less, preferably in an amount of 0.2 % by mass or less, preferably in an amount of 0.1 % by mass or less, preferably in an amount of 0.05 % by mass or less, preferably in an amount of 0.01 % by mass or less.
19. The aluminium alloy according to any one of items 1 to 18, wherein Co is present in an amount of 0.3 % by mass or less, preferably in an amount of 0.2 % by mass or less, preferably in an amount of 0.1 % by mass or less, preferably in an amount of 0.05 % by mass or less, preferably in an amount of 0.01 % by mass or less.
20. The aluminium alloy according to any one of items 1 to 19, wherein the aluminium alloy optionally further comprises at least one element, wherein each of said elements is present in an amount of from 0 to 0.5 % by mass, preferably in an amount of from 0 to 0.2 % by mass, preferably of from 0 to 0.1 % by mass, preferably of from 0 to 0.05 % by mass, and wherein the at least one element is selected from the group consisting of Molybdenum (Mo), Hafnium (Hf), Calcium (Ca), Gallium (Ga), Scandium (Sc), Niobium (Nb), and Cerium (Ce).
21. The aluminium alloy according to any one of items 1 to 20, comprising
   a) of from 6 to 12 % by mass of magnesium (Mg);
   b) of from 0.01 to 0.4 % by mass of titanium (Ti);
   c) of from 0.002 to 0.08 % by mass of boron (B);
   d) of from 0.002 to 0.1 % by mass of beryllium (Be);
   e) of from 0 to 0.5 % by mass of manganese (Mn);
   f) of from 0 to 0.1 % by mass of iron (Fe);
   g) of from 0 to 2.5 % by mass of zinc (Zn);
   h) of from 0 to 0.5 % by mass of chromium (Cr);
   i) of from 0 to 0.5 % by mass of zirconium (Zr);
   j) of from 0 to 0.25 % by mass of vanadium (V);
   k) of from 0 to 0.05 % by mass of copper (Cu);
   l) of from 0 to 0.6 % by mass of silicon (Si);
   m) of from 0 to 0.5 % by mass of nickel (Ni);
   n) of from 0 to 0.3 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
22. The aluminium alloy according to any one of items 1 to 20, comprising
   a) of from 6.5 to 12 % by mass of magnesium (Mg);
   b) of from 0.015 to 0.15 % by mass of titanium (Ti);
   c) of from 0.003 to 0.03 % by mass of boron (B);
   d) of from 0.003 to 0.1 % by mass of beryllium (Be);
   e) of from 0 to 1 % by mass of manganese (Mn);
   f) of from 0 to 0.1 % by mass of iron (Fe);
   g) of from 0 to 2.5 % by mass of zinc (Zn);
   h) of from 0 to 0.2 % by mass of chromium (Cr);
   i) of from 0 to 0.2 % by mass of zirconium (Zr);
   j) of from 0 to 0.1 % by mass of vanadium (V);
   k) of from 0 to 0.05 % by mass of copper (Cu);
   l) of from 0 to 0.5 % by mass of silicon (Si);
   m) of from 0 to 0.5 % by mass of nickel (Ni);
   n) of from 0 to 0.3 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
23. The aluminium alloy according to any one of items 1 to 20, comprising
   a) of from 6 to 10 % by mass of magnesium (Mg);
   b) of from 0.01 to 0.2 % by mass of titanium (Ti);
   c) of from 0.002 to 0.04 % by mass of boron (B);
   d) of from 0.003 to 0.1 % by mass of beryllium (Be);
   e) of from 0 to 1 % by mass of manganese (Mn);
   f) of from 0 to 0.1 % by mass of iron (Fe);
   g) of from 0 to 2.5 % by mass of zinc (Zn);
   h) of from 0 to 0.2 % by mass of chromium (Cr);
   i) of from 0 to 0.2 % by mass of zirconium (Zr);
   j) of from 0 to 0.1 % by mass of vanadium (V);
   k) of from 0 to 0.05 % by mass of copper (Cu);
   l) of from 0 to 0.6 % by mass of silicon (Si);
   m) of from 0 to 0.1 % by mass of nickel (Ni);
   n) of from 0 to 0.1 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
24. The aluminium alloy according to any one of items 1 to 20, comprising
   a) of from 7 to 9 % by mass of magnesium (Mg);
   b) of from 0.015 to 0.15 % by mass of titanium (Ti);
   c) of from 0.003 to 0.03 % by mass of boron (B);
   d) of from 0.004 to 0.05 % by mass of beryllium (Be);
   e) of from 0 to 0.1 % by mass of manganese (Mn);
   f) of from 0 to 0.1 % by mass of iron (Fe);
   g) of from 0 to 1 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.05 % by mass of copper (Cu);
   l) of from 0 to 0.4 % by mass of silicon (Si);
   m) of from 0 to 0.5 % by mass of nickel (Ni);
   n) of from 0 to 0.3 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
25. The aluminium alloy according to any one of items 1 to 20, comprising
   a) of from 7.5 to 8.5 % by mass of magnesium (Mg);
   b) of from 0.015 to 0.15 % by mass of titanium (Ti);
   c) of from 0.003 to 0.03 % by mass of boron (B);
   d) of from 0.004 to 0.05 % by mass of beryllium (Be);
   e) of from 0 to 0.1 % by mass of manganese (Mn);
   f) of from 0 to 0.1 % by mass of iron (Fe);
   g) of from 0 to 1 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.05 % by mass of copper (Cu);
   l) of from 0 to 0.4 % by mass of silicon (Si);
   m) of from 0 to 0.5 % by mass of nickel (Ni);
   n) of from 0 to 0.3 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
26. The aluminium alloy according to any one of items 1 to 20, comprising
   a) of from 7.5 to 8.5 % by mass of magnesium (Mg);
   b) of from 0.015 to 0.1 % by mass of titanium (Ti);
   c) of from 0.003 to 0.03 % by mass of boron (B);
   d) of from 0.004 to 0.05 % by mass of beryllium (Be);
   e) of from 0 to 0.05 % by mass of manganese (Mn);
   f) of from 0.01 to 0.1 % by mass of iron (Fe);
   g) of from 0 to 0.5 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.03 % by mass of copper (Cu);
   l) of from 0 to 0.3 % by mass of silicon (Si);
   m) of from 0 to 0.2 % by mass of nickel (Ni);
   n) of from 0 to 0.1 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
27. The aluminium alloy according to any one of items 1 to 20, comprising
   a) of from 7.5 to 8.5 % by mass of magnesium (Mg);
   b) of from 0.015 to 0.1 % by mass of titanium (Ti);
   c) of from 0.003 to 0.03 % by mass of boron (B);
   d) of from 0.005 to 0.02 % by mass of beryllium (Be);
   e) of from 0 to 0.05 % by mass of manganese (Mn);
   f) of from 0.01 to 0.1 % by mass of iron (Fe);
   g) of from 0 to 0.1 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.03 % by mass of copper (Cu);
   l) of from 0 to 0.15 % by mass of silicon (Si);
   m) of from 0 to 0.1 % by mass of nickel (Ni);
   of from 0 to 0.05 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
28. The aluminium alloy according to any one of items 1 to 20, comprising
   a) of from 7.5 to 8.5 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.03 % by mass of copper (Cu);
   l) of from 0 to 0.15 % by mass of silicon (Si);
   m) of from 0 to 0.05 % by mass of nickel (Ni);
   n) of from 0 to 0.05 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
29. The aluminium alloy according to any one of items 1 to 20, comprising
   a) of from 7.5 to 8.5 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
30. The aluminium alloy according to any one of items 1 to 20, comprising
   a) of from 8 to 8.5 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
31. The aluminium alloy according to any one of items 1 to 20, comprising
   a) of from 8 to 12 % by mass of magnesium (Mg);
   b) of from 0.015 to 0.15 % by mass of titanium (Ti);
   c) of from 0.003 to 0.03 % by mass of boron (B);
   d) of from 0.004 to 0.05 % by mass of beryllium (Be);
   e) of from 0 to 0.1 % by mass of manganese (Mn);
   f) of from 0 to 0.1 % by mass of iron (Fe);
   g) of from 0 to 1 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.05 % by mass of copper (Cu);
   l) of from 0 to 0.4 % by mass of silicon (Si);
   m) of from 0 to 0.5 % by mass of nickel (Ni);
   n) of from 0 to 0.3 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
32. The aluminium alloy according to any one of items 1 to 20, comprising
   a) of from 8 to 12 % by mass of magnesium (Mg);
   b) of from 0.015 to 0.1 % by mass of titanium (Ti);
   c) of from 0.003 to 0.03 % by mass of boron (B);
   d) of from 0.004 to 0.05 % by mass of beryllium (Be);
   e) of from 0 to 0.05 % by mass of manganese (Mn);
   f) of from 0.01 to 0.1 % by mass of iron (Fe);
   g) of from 0 to 0.5 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.03 % by mass of copper (Cu);
   l) of from 0 to 0.3 % by mass of silicon (Si);
   m) of from 0 to 0.2 % by mass of nickel (Ni);
   n) of from 0 to 0.1 % by mass of cobalt (Co)
   wherein the aluminium alloy further comprises inevitable impurities; with the balance being aluminium (Al); each in relation to the total mass of the alloy composition, and wherein all compounds of the alloy add up to a total of 100 % by mass.
33. The aluminium alloy according to any one of items 1 to 20, comprising
   a) of from 8 to 12 % by mass of magnesium (Mg);
   b) of from 0.015 to 0.1 % by mass of titanium (Ti);
   c) of from 0.003 to 0.03 % by mass of boron (B);
   d) of from 0.005 to 0.02 % by mass of beryllium (Be);
   e) of from 0 to 0.05 % by mass of manganese (Mn);
   f) of from 0.01 to 0.1 % by mass of iron (Fe);
   g) of from 0 to 0.1 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.03 % by mass of copper (Cu);
   l) of from 0 to 0.15 % by mass of silicon (Si);
   m) of from 0 to 0.1 % by mass of nickel (Ni);
   of from 0 to 0.05 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
34. The aluminium alloy according to any one of items 1 to 20, comprising
   a) of from 9 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.05 % by mass of chromium (Cr);
   i) of from 0 to 0.05 % by mass of zirconium (Zr);
   j) of from 0 to 0.05 % by mass of vanadium (V);
   k) of from 0 to 0.03 % by mass of copper (Cu);
   l) of from 0 to 0.15 % by mass of silicon (Si);
   m) of from 0 to 0.05 % by mass of nickel (Ni);
   n) of from 0 to 0.05 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
35. The aluminium alloy according to any one of items 1 to 20, comprising
   a) of from 9.5 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
36. The aluminium alloy according to any one of items 1 to 20, comprising
   a) of from 9.5 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
37. The aluminium alloy according to any one of items 1 to 20, comprising
   a) of from 10 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
38. The aluminium alloy according to any one of items 1 to 20, comprising
   a) of from 11 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
39. The aluminium alloy according to any one of items 1 to 20, comprising
   a) of from 11 to 11.5 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
40. The aluminium alloy according to any one of items 1 to 20, comprising
   a) of from 6.5 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
41. The aluminium alloy according to any one of items 1 to 20, comprising
   a) of from 7 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
42. The aluminium alloy according to any one of items 1 to 20, comprising
   a) of from 7.5 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
43. The aluminium alloy according to any one of items 1 to 20, comprising
   a) of from 8 to 12 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
44. The aluminium alloy according to any one of items 1 to 20, comprising
   a) of from 8 to 11.5 % by mass of magnesium (Mg);
   b) of from 0.015 to 0.08 % by mass of titanium (Ti);
   c) of from 0.003 to 0.016 % by mass of boron (B);
   d) of from 0.005 to 0.02 % by mass of beryllium (Be);
   e) of from 0 to 0.01 % by mass of manganese (Mn);
   f) of from 0.05 to 0.09 % by mass of iron (Fe);
   g) of from 0 to 0.05 % by mass of zinc (Zn);
   h) of from 0 to 0.01 % by mass of chromium (Cr);
   i) of from 0 to 0.01 % by mass of zirconium (Zr);
   j) of from 0 to 0.01 % by mass of vanadium (V);
   k) of from 0 to 0.01 % by mass of copper (Cu);
   l) of from 0 to 0.1 % by mass of silicon (Si);
   m) of from 0 to 0.01 % by mass of nickel (Ni);
   n) of from 0 to 0.01 % by mass of cobalt (Co);
   wherein the aluminium alloy further comprises inevitable impurities; with the balance being aluminium (Al); each in relation to the total mass of the alloy composition, and wherein all compounds of the alloy add up to a total of 100 % by mass.
45. Aluminium alloy product comprising an aluminium alloy according to any one of items 1 to 44, wherein the aluminium alloy product is an extruded aluminium profile.
46. Method for the manufacture of an aluminium alloy according to any one of items 1 to 44, comprising the steps of
   a. Providing a raw aluminium;
   b. Heating the raw aluminium to a temperature in the range of from 650 to 850 °C, preferably from 750 to 800 °C;
   c. Adding Mg and Be to result in a raw alloy;
   d. Optionally degassing the raw alloy;
   e. Adding Ti and B to the optionally degassed raw alloy to prepare the aluminium alloy; and
   f. Casting the aluminium alloy to prepare an aluminium billet.
47. Method for the manufacture of an aluminium alloy product according to item 45, wherein the manufacture of the aluminium alloy product comprises the steps of
   g. Preheating an aluminium billet consisting of an aluminium alloy according to any one of items 1 to 20, to a temperature in the range of from 400 °C to 450 °C, preferably in the range of from 420 °C to 440 °C, to result in a preheated aluminium billet;
   h. Inserting the preheated aluminium billet from step g) into an extrusion press;
   i. Extruding the preheated aluminium billet to result an extruded aluminium profile.
48. Method for the manufacture of an aluminium ally product according to item 47, wherein extruding the preheated aluminium billet in step i) is carried out at a maximum force in the range of from 5,000 to 15,000 kN, preferably form 7,000 to 12,000 kN, more preferably 8,000 to 10,000 kN, most preferably at a maximum force of about 9,000 kN.
49. The method according to item 47 or 48, wherein the method further comprises the step of
   j. heat treating the extruded aluminium profile by heating the extruded aluminium profile at a temperature of at least 380 °C, or at least 400 °C, or at least 430 °C, or at least 450 °C, for a period of less than 1 hour, or less than 3 hours, or less than 5 hours, or less than 8 hours, or less than 12 hours, or less than 18 hours, or less than 24 hours, preferably less than 12 hours, or preferably less than 18 hours, or for a period of at least 10 minutes, or at least 1 hour, or at least 3 hours, or at least 8 hours, or at least 12 hours, or at least 24 hours, and then cooled in air at ambient temperature.
50. Extruded aluminium profile prepared by a method according to any one of items 47 to 49.
51. The extruded aluminium profile according to any one of items 45 or 50, wherein the extruded aluminium profile is an extruded aluminium hollow profile.
52. The extruded aluminium profile according to any one of items 45, and 50 to 51, wherein at least parts of the extruded aluminium profile have a thickness in the range of from 1 to 15 mm, preferably 1 to 10 mm, preferably from 2 to 8 mm, preferably from 2 to 6 mm; or 2 to 5 mm, preferably 2.5 to 4 mm.
53. The extruded aluminium profile according to any one of items 45, and 50 to 52, wherein the aluminium alloy of the extruded aluminium profile has a tensile strength Rₘ of at least 260 MPa, preferably at least 280 MPa, preferably at least 300 MPa, preferably at least 320 MPa, preferably at least 350 MPa.
54. The extruded aluminium profile according to any one of items 45, and 50 to 53, wherein the aluminium alloy of the extruded aluminium profile has a yield strength R_{p0,2} of at least 100 MPa, preferably at least 140 MPa, preferably at least 180 MPa, preferably at least 190 MPa.
55. The extruded aluminium profile according to any one of items 45, and 50 to 54, wherein the aluminium alloy of the extruded aluminium profile has an elongation A of at least 15 %, preferably at least 20 %, further preferably at least 25 %, further preferably at least 30 %, further preferably at least 40 %, most preferably at least 45 %.
56. The extruded aluminium profile according to any one of items 45, and 50 to 55, wherein the aluminium alloy of the extruded aluminium profile has a ratio X between the elongation A and the tensile strength Rₘ of at least 0.05 %/MPa, preferably at least 0.07 %/MPa, preferably at least 0.09 %/MPa, preferably at least 0.11 %/MPa, preferably at least 0.13 %/MPa, preferably at least 0.15 %/MPa, preferably at least 0.17 %/MPa.
57. Use of an aluminium alloy according to any one of items 1 to 44 in an extrusion process or a wrought process.

## Claims

1. An aluminium alloy comprising
a) of from 6 to 12 % by mass of magnesium (Mg);
b) of from 0.01 to 0.5 % by mass of titanium (Ti);
c) of from 0.001 to 0.1 % by mass of boron (B);
d) of from 0.002 to 0.2 % by mass of beryllium (Be);
e) of from 0 to 2.5 % by mass of manganese (Mn);
f) of from 0 to 0.2 % by mass of iron (Fe);
g) of from 0 to 5 % by mass of zinc (Zn);
h) of from 0 to 1 % by mass of chromium (Cr);
i) of from 0 to 1 % by mass of zirconium (Zr);
j) of from 0 to 0.5 % by mass of vanadium (V);
k) of from 0 to 0.06 % by mass of copper (Cu);
l) of from 0 to 1 % by mass of silicon (Si);
m) of from 0 to 1 % by mass of nickel (Ni);
n) of from 0 to 0.5 % by mass of cobalt (Co);
wherein the aluminium alloy further comprises inevitable impurities;
with the balance being aluminium (Al); each amount in relation to the total mass of the alloy composition, and wherein all compounds of the alloy add up to a total of 100 % by mass.

2. The aluminium alloy according to claim 1, wherein the aluminium alloy is suitable for extrusion and/or wrought applications.

3. The aluminium alloy according to any one of claims 1 or 2, wherein Mg is present in an amount of from 6.5 to 12 % by mass, preferably in an amount of from 7 to 12 % by mass, preferably in an amount of from 7.5 to 12 % by mass, preferably in an amount of from 8 to 12 % by mass, preferably in an amount of from 8 to 11.5 % by mass.

4. The aluminium alloy according to any one of claims 1 to 3, wherein Ti is present
i) in an amount of from 0.01 to 0.4 % by mass, preferably in an amount of from 0.01 to 0.3 % by mass, preferably in an amount of from 0.01 to 0.2 % by mass, preferably in an amount of from 0.015 to 0.15 % by mass, preferably in an amount of from 0.015 to 0.1 % by mass; preferably in an amount of from 0.015 to 0.08 % by mass; and/or
ii) in an amount of from 0.4 % by mass or less, preferably in an amount of 0.3 % by mass or less, preferably in an amount of 0.2 % by mass or less, preferably in an amount of 0.15 % by mass or less, preferably in an amount of 0.1 % by mass or less; preferably in an amount of 0.08 % by mass or less; and/or
iii) in an amount of 0.01 % by mass or more, preferably in an amount of 0.015 % by mass or more.

5. The aluminium alloy according to any one of claims 1 to 4, wherein Be is present
i) in an amount of from 0.002 to 0.15 % by mass, preferably in an amount of from 0.003 to 0.1 % by mass, preferably in an amount of from 0.004 to 0.05 % by mass, preferably in an amount of from 0.005 to 0.02 % by mass; and/or
ii) in an amount of 0.002 % by mass or more, or in an amount of 0.003 % by mass or more, or in an amount of 0.004 % by mass or more, or in an amount of 0.005 % by mass or more, or in an amount of 0.015 % by mass or more; and/or
iii) in an amount of 0.15 % by mass or less, or in an amount of 0.1 % by mass or less, or in an amount of 0.05 % by mass or less, or in an amount of 0.02 % by mass or less.

6. The aluminium alloy according to any one of claims 1 to 5, wherein B is present
i) in an amount of from 0.002 to 0.08 % by mass, preferably in an amount of from 0.002 to 0.06 % by mass, preferably in an amount of from 0.002 to 0.04 % by mass, preferably in an amount of from 0.003 to 0.02 % by mass, preferably in an amount of from 0.003 to 0.016 % by mass; and/or
ii) in an amount of 0.002 % by mass or more, or in an amount of 0.0025 % by mass or more, or in an amount of 0.003 % by mass or more; and/or
iii) in an amount of 0.08 % by mass or less, or in an amount of 0.06 % by mass or less, or in an amount of 0.04 % by mass or less, or in an amount of 0.02 % by mass or less, or in an amount of 0.016 % by mass or less.

7. Aluminium alloy product comprising an aluminium alloy according to any one of claims 1 to 6, wherein the aluminium alloy product is an extruded aluminium profile.

8. Method for the manufacture of an aluminium alloy according to any one of claims 1 to 6, comprising the steps of
a) Providing a raw aluminium;
b) Heating the raw aluminium to a temperature in the range of from 650 to 850 °C, preferably from 750 to 800 °C;
c) Adding Mg and Be to result in a raw alloy;
d) Optionally degassing the raw alloy;
e) Adding Ti and B to the optionally degassed raw alloy to prepare the aluminium alloy; and
f) Casting the aluminium alloy to prepare an aluminium billet.

9. Method for the manufacture of an aluminium alloy product according to claim 7, wherein the manufacture of the aluminium alloy product comprises the steps of
g) Preheating an aluminium billet consisting of an aluminium alloy according to any one of claims 1 to 6, to a temperature in the range of from 400 °C to 450 °C, preferably in the range of from 420 °C to 440 °C, to result in a preheated aluminium billet;
h) Inserting the preheated aluminium billet from step g) into an extrusion press;
i) Extruding the preheated aluminium billet to result an extruded aluminium profile.

10. The method according to claim 9, wherein extruding the preheated aluminium billet in step i) is carried out at a maximum force in the range of from 5,000 to 15,000 kN, preferably form 7,000 to 12,000 kN, more preferably 8,000 to 10,000 kN, most preferably at a maximum force of about 9,000 kN.

11. The method according to claim 9 or 10, wherein the method further comprises the step of
j) heat treating the extruded aluminium profile by heating the extruded aluminium profile at a temperature of at least 380 °C, or at least 400 °C, or at least 430 °C, or at least 450 °C, for a period of less than 1 hour, or less than 3 hours, or less than 5 hours, or less than 8 hours, or less than 12 hours, or less than 18 hours, or less than 24 hours, preferably less than 12 hours, or preferably less than 18 hours, or for a period of at least 10 minutes, or at least 1 hour, or at least 3 hours, or at least 8 hours, or at least 12 hours, or at least 24 hours, and then cooled in air at ambient temperature.

12. Extruded aluminium profile prepared by a method according to any one of claims 9 to 11.

13. The extruded aluminium profile according to any one of claims 7 or 12, wherein the extruded aluminium profile is an extruded aluminium hollow profile, preferably wherein at least parts of the extruded aluminium profile have a thickness in the range of from 1 to 15 mm, preferably 1 to 10 mm, preferably from 2 to 8 mm, preferably from 2 to 6 mm; or 2 to 5 mm, preferably 2.5 to 4 mm.

14. The extruded aluminium profile according to any one of claims 7, and 12 or 13, wherein the aluminium alloy of the extruded aluminium profile has a tensile strength Rₘ of at least 260 MPa, preferably at least 280 MPa, preferably at least 300 MPa, preferably at least 320 MPa, preferably at least 350 MPa; and/or
wherein the aluminium alloy of the extruded aluminium profile has a yield strength R_{p0,2} of at least 100 MPa, preferably at least 140 MPa, preferably at least 180 MPa, preferably at least 190 MPa; and/or
wherein the aluminium alloy of the extruded aluminium profile has an elongation A of at least 15 %, preferably at least 20 %, further preferably at least 25 %, further preferably at least 30 %, further preferably at least 40 %, most preferably at least 45 %; and/or wherein the aluminium alloy of the extruded aluminium profile has a ratio X between the elongation A and the tensile strength Rₘ of at least 0.05 %/MPa, preferably at least 0.07 %/MPa, preferably at least 0.09 %/MPa, preferably at least 0.11 %/MPa, preferably at least 0.13 %/MPa, preferably at least 0.15 %/MPa, preferably at least 0.17 %/MPa.

15. Use of an aluminium alloy according to any one of claims 1 to 6 in an extrusion process or a wrought process.
